

Jan. 22, 1952

W. E. BRILL

2,582,946

FLAME METHOD OF CUTTING METAL

Filed June 21, 1948



Fig. 1



Fig. 2



Fig. 3

Fig. 4



Fig. 5

Fig. 6

INVENTOR  
Warren E. Brill  
BY Rodnick Malcolm

ATTORNEY

## UNITED STATES PATENT OFFICE

2,582,946

## FLAME METHOD OF CUTTING METAL

Warren E. Brill, Haddon Heights, N. J.

Application June 21, 1948, Serial No. 34,238

5 Claims. (Cl. 148—9)

1

This invention relates to the art of subjecting metal to the action of heat supplied by an oxy-acetylene (or similar) flame for the purpose of melting, cutting, severing, gouging, beveling, cleansing or inspecting the metal.

The conventional oxy-acetylene process of "cutting" ferrous metals depends for its operation upon the rapid chemical action between the white-hot metal and a stream of pure oxygen. Thus, while the prior art is replete with cutting torches, all such tools may be said to consist, essentially, of a blowpipe having a nozzle from which there emerges (1) a flame consisting of a mixture of acetylene (propane or other fuel gas) and oxygen, usually in the proportion of one-to-one, capable of heating a spot on the iron or steel to a white-hot temperature and (2) a discrete stream of substantially pure oxygen, under pressure.

In the hands of a skilled workman modern oxy-acetylene torches are susceptible of many uses. Thus, they may be employed in cutting through even the thickest steel, in piercing holes in iron or steel and also in beveling and gouging operations upon ferrous plate or pipe stock. The use of present-day torches, however, is subject to certain limitations. By way of example, such torches can be used only upon ferrous metals since, as is well known, non-ferrous metals do not form oxides that will ignite when subjected to the high-pressure oxygen stream.

Accordingly, it is an object of the present invention to provide a novel method of cutting both ferrous and non-ferrous metals.

Another limitation upon the use of present day torches is manifest in the cutting of high carbon steel. Here the oxygen stream from the high pressure valve has a rapid cooling action upon the hot metal. As a result of this rapid cooling action numerous small cracks are formed in the metal adjacent to the cut. Therefore, in cutting away the riser or sprue of a casting constituted of high carbon steel the cut must be made a substantial distance from the body of the casting so that the said cracks will be confined to a stub which, subsequently, must be machined off, as on a lathe. The high cost of machining-away a large stub frequently dictates the use of forged-metal in instances where cast-metal might be used were it not for the trouble and expense of removing the riser or sprue from the casting.

Accordingly, another object of the invention is to provide an improved "flame" method of cutting high carbon steel, and one which may be practiced without producing cracks or other defects in said metal.

Another very real objection to present day oxy-acetylene torches is that they are incapable of that nice degree of control which would permit their use in the removal, say, of boiler tubes or

2

rivets, without danger of scoring or otherwise scarring the metal in which such parts are usually seated. The same lack of control imposes a lower limit (say  $\frac{3}{8}$  of an inch) upon the thickness of the metal which can be subjected to the cutting or gouging action of a conventional torch.

Accordingly, another object of the present invention is to provide a method which shall lend itself readily to the removal of metal from stock of substantially any thickness dimension, and this too without deleterious effects upon the surrounding metal in the event of an accidental or temporary loss of control of the torch while it is in use.

Yet another object of the present invention is to provide a novel method of making an "on-the-spot" inspection of welded metal.

In the above connection it will be recalled that, up to now, the only means available for revealing sub-surface defects in welded metal comprise

(a) X-rays and (b) so-called "supersonic" or vibratile methods. The limitations upon the use of such test methods and equipments are so serious that, as a practical matter, the only weld-insurance that is acceptable to large-scale users

of welded metal is the high standards which they have established as to the skill and experience of the persons entrusted with making the welds. As will hereinafter more fully appear, the present invention by providing a simple and convenient

method for making a non-destructive (or easily repairable) sub-surface exploration of the metal, permits the use of welding in instances where welding has not heretofore been used because of the absence of a satisfactorily convenient means of inspecting the metal after it has been welded.

Another and important object of the invention is to provide a truly "low" pressure "flame" method for the cutting etc. of metal, and thus to effect substantial savings not only in operating expenses but also in the cost and weight of the torch and its accessories.

The foregoing and other objects are achieved in accordance with the method of the present invention by mixing oxygen and acetylene (propane, or other fuel gas) in the proportions required to provide a "neutral" flame, when the mixture is ignited, then subjecting the surface metal to be cut to said flame for a period sufficiently long to provide a drop or small puddle of

molten metal upon said surface and then increasing the force or pressure back of the flame (as by controllably increasing the amount and pressure of the oxygen in the mix) in order to blow the molten metal away, from its area of origin, without burning it or scoring the surrounding metal.

As will hereinafter more fully appear in connection with the description of the accompanying drawings, a conventional "cutting torch"

(i. e. one having a lever actuated, "high-pressure" oxygen valve) may be modified to permit the practice of the method of the invention by (a) blocking the opening through which the "high pressure" oxygen stream normally passes to the central nozzle opening, (b) using said "high pressure" valve to control a "low pressure" stream of oxygen and (c) diverting said "low pressure" stream either within the torch or its nozzle, to the passageway through which the mixed oxygen and fuel gas flow. Alternatively, the method of the present invention may be practiced with a conventional cutting torch by providing the torch with a "welding" nozzle (i. e. one having a single orifice) with its seat cut away in a manner later described.

Certain preferred details of construction and operation together with other objects and advantages will appear and the invention itself will be best understood upon reference to the following specification and to the accompanying drawing wherein:

Fig. 1 is a side elevation and Fig. 2 is a longitudinal sectional view of a cutting blowpipe constructed in accordance with the principle of the invention.

Fig. 3 is a longitudinal section of an alternative form of blowpipe and nozzle within the invention.

Fig. 4 is a plan view showing the tip end of the nozzle of Fig. 3.

Fig. 5 shows a "neutral" flame and Fig. 6 shows a "highly oxidizing" flame emerging from the nozzle of Fig. 2 and

Fig. 7 is a view in perspective showing the manner in which the blowpipe of the invention operates to "cut" a piece of metal.

The blowpipe used in the method of the present invention, as it is illustrated in Fig. 1, has the outward appearance of a conventional "cutting torch," in that it has a cylindrical body 1 which terminates at one end in a nozzle 2 and at its opposite end in a valve block 3. As is conventional, the valve block 3 is provided with an inlet nipple 4 through which acetylene or other fuel gas enters a pipe 5 (Fig. 2) within the body 1 under the control of a handwheel 6, and a second nipple 7 through which oxygen is supplied to two oxygen pipes 8 and 10 under the control of a handwheel 9 and lever 11, respectively. If desired separate inlet connections may be provided for the two oxygen pipes 8 and 10.

As is also conventional, the oxygen inlet pipe 8 extends a limited distance through the interior of the inlet pipe 5 for the fuel gas and terminates in an injector or "mixing chamber" 12 where the said gases are mixed, preferably in the proportion of one-to-one, solely under the "set" control of the handwheels 6 and 9, respectively.

In accordance with the present invention the combustible mixture in the injector or mixing chamber 12 instead of passing directly to the so-called "pre-heat orifices" of a conventional "cutting nozzle" passes through a combustible-mixture passageway 13 to a second chamber 14 adjacent to the nozzle end of the blowpipe where the percentage and pressure of the oxygen in the mixture, and hence of the force or pressure "in back of the flame," may be increased by the addition to the mix of oxygen supplied under the control of the lever-actuated valve 11 in the second oxygen inlet pipe 10. As previously indicated, the degree to which the force or pressure in back of the flame need be increased in the practice of the method of the present invention

is very small and, ordinarily, need be no more than a pound or two. Hence the hose and other equipment used in the practice of the invention may be of light weight, yet safely-portable, construction.

In the embodiment of the torch shown in Figs. 1 and 2 the nozzle 2 contains but a single opening 2a through which the combustible mixture or mixtures in the chamber 14 pass. Alternatively, as shown in Figs. 3 and 4, when a flame of a greater circumference is required, the nozzle which is here designated 2' may be provided with several circumferentially arranged openings 2b, 2c etc. A nozzle similar to the one shown in Figs. 3 and 4 may be made from a conventional cutting-nozzle simply by plugging its central orifice and cutting-off (or cutting a passageway through) the end of the seat (indicated by the dotted lines 14', Fig. 3) through which the "cutting oxygen" ordinarily passes to the said central orifice. With the nozzle thus altered it may be used with a conventional "cutting torch" in the practice of the present invention, since the space formerly occupied by the said seat now comprises a mixing chamber similar in function to the "second" mixing chamber 14 of the blowpipe shown in Fig. 2.

As previously indicated, the present invention provides a method of "cutting" metal which comprises the steps: (a) of subjecting a small area or spot on the exposed surface of the metal to a flame of a temperature and pressure calculated to convert the said spot into a stationary drop or puddle of molten metal and (b) increasing the pressure or force of the flame (as by increasing the amount and pressure of the oxygen in the combustible mixture) to a degree sufficient to blow away, or to merely "upset," the said drop of molten metal.

The flame to which the metal is first subjected preferably, but not necessarily, comprises a so-called "neutral" flame i. e. one wherein the gases emerging from the tip of the nozzle comprise a one-to-one mixture of fuel gas and oxygen. Such a mixture may be achieved by manipulating the handwheels (6 and 9) of the blowpipe until the clearly defined inner cone c (see Fig. 5) characteristic of a neutral flame is achieved. The clearly defined inner cone of a neutral flame is from one-sixteenth to one inch long, depending upon the dimensions of the nozzle openings. If the size of the nozzle openings is increased, a larger flame will be produced since more of the combustible mixture can pass therethrough in a given time.

The alteration in the pressure or intensity of the flame required to "blow away" the molten metal produced by the "neutral" flame is obtained by pressing down the conveniently located lever 11 that controls the admission of pure oxygen into the "second" mixing chamber 14. The increase in the force or pressure back of the flame which results from pressing down the hand lever 11 will ordinarily convert the "neutral" flame (Fig. 5) into one having the shorter cone c' (Fig. 6) characteristic of a "highly oxidizing" flame. The upper limit of the pressure increase may be fixed at the regulator (not shown) of the oxygen supply. If the regulator is set to pass say 12 lbs. and the hand wheel 9, when set to provide a neutral flame at 10 lbs. pressure, then, when the lever 11 is pressed down, the additional oxygen supplied to the mix can be no more than two pounds, making 12 lbs. in all. This increase in the pressure of the combustible mixture is not

believed necessarily to be accompanied by any substantial change in the temperature of the flame. That is to say, the temperature of the flame remains sufficiently high to melt the metal, and yet is not so high as to "burn" the metal or convert it into "slag." In any event the flame has no cooling action on the surrounding metal such as accompanies the release of the stream of "cutting oxygen" from a conventional cutting torch. Hence the present invention can be used upon high carbon steel without producing cracks adjacent to the cut.

The technique involved in the cutting of metal in accordance with the method of the present invention is similar to that employed by welders in "carrying a puddle" across the surface of a piece of steel. Thus, referring to Fig. 7, when a "puddle" of molten metal has been created on the surface of the metal M to be cut by the action of the "neutral" flame emanating from the nozzle (which may be of any convenient shape), and the pressure back of the flame has been increased (by pressing down the lever 11, Figs. 1 and 2), the nozzle is moved slowly over the surface of the cut. The said increase in pressure is sufficient to blow the molten metal, gently outwardly, usually on both sides of the cut and to deposit it in the form of a friable deposit which may subsequently be brushed away. Since the temperature of the flame is not decreased by the described increase in the pressure or force of the flame, a fresh supply of molten metal is constantly presented to the nozzle. Should the puddle be "lost," as it may be if the torch is moved too rapidly, the operator returns the nozzle to the point where the cutting action ceased and creates a new puddle, preferably by letting-up on the hand lever 11.

The gentle "blowing away" of the molten metal when the velocity of the flame or jet is increased by pressing down upon the lever 11 permits the torch of the present invention to be used in instances where the high pressure blast of the un-ignited oxygen from a conventional cutting torch could not be tolerated. One such use is the removal of tubes from a boiler for purposes of replacement. Here a conventional cutting torch cannot be used because of danger of scoring the boiler plates with the cold oxygen blast. Obviously, the use of the torch of the present invention presents no such hazard even in the hands of a careless workman. Similarly, if an attempt were to be made to use a conventional cutting torch to detect subsurface defects in welded metal, the high pressure oxygen blast might blow away the metal containing the defect which is intended to be exposed. On the other hand the absence of any "blasting" action in the use of the torch of the present invention permits the removal of even the thinnest layer of metal without risk of damaging the underlying or surrounding metal.

From the foregoing, it will now be apparent that the present invention provides a novel and economical "flame" method of subjecting metal to the action heat supplied by an oxy-acetylene or similar flame for the purpose of melting, cutting, severing, gouging, beveling or inspecting the same.

#### What is claimed is:

1. A method of cutting metal which consists in subjecting a surface portion of said metal to a flame produced by the ignition of a substantially uniform mixture of oxygen and a fuel gas for a period of time sufficiently long to create a

puddle of molten metal on said surface, and then increasing the pressure of said substantially uniform mixture of gases feeding said flame to a degree sufficient to move said puddle of molten metal away from its area of origin.

2. A method of cutting metal which consists in subjecting a surface portion of said metal to a flame produced by the ignition of a substantially uniform mixture of oxygen and a fuel gas, said flame being of a temperature and pressure sufficient to generate a puddle of molten metal on said surface, then increasing the pressure of said substantially uniform mixture of gases feeding said flame to a degree sufficient to blow said molten metal away from said surface portion, and then moving said flame along the part of the metal to be cut while maintaining the temperature of said flame sufficiently high to render said part of said metal molten.

20 3. The method of cutting metal which consists in subjecting a local area of the metal to be cut to a "neutral" flame, consisting of a substantially uniform mixture of oxygen and acetylene, for a period of time sufficiently long to convert the metal of which said local area is comprised into a puddle of molten metal, and then converting said "neutral" flame into a "highly oxidizing" flame consisting of a substantially uniform mixture of oxygen and acetylene of a pressure sufficiently high to move said molten metal away from said local area.

4. The method of cutting a metallic body which consists in forming an ignited combustible gas jet of low velocity, directing said low-velocity jet upon the metallic surface of the body for a period sufficiently long to convert a small area of said surface into molten metal, forming an ignited gas jet consisting of a substantially uniform mixture of oxygen and fuel gas of a velocity greater than that of said first mentioned jet, and directing said second mentioned jet upon said molten metal whereby to blow said molten metal away from said surface area.

5. The invention as set forth in claim 4 and 45 wherein the temperature of said first and said second-mentioned combustible-gas jets are of the same general order, whereby the cooling effect of said second-mentioned jet upon said metal is minimized.

50 WARREN E. BRILL.

#### REFERENCES CITED

The following references are of record in the file of this patent:

#### 55 UNITED STATES PATENTS

|    | Number    | Name           | Date           |
|----|-----------|----------------|----------------|
| 60 | 703,940   | Menne          | July 1, 1902   |
|    | 866,866   | Jotstrand      | Sept. 24, 1907 |
|    | 1,311,815 | Harris         | July 29, 1919  |
|    | 1,519,582 | Harris         | Dec. 16, 1924  |
|    | 2,210,403 | Skinner        | Aug. 6, 1940   |
|    | 2,367,316 | Skinner        | Jan. 16, 1945  |
|    | 2,425,709 | Bucknam et al. | Aug. 19, 1947  |
| 65 | 2,441,179 | Anderson       | May 11, 1948   |

#### OTHER REFERENCES

The Oxy-Acetylene Handbook, 3rd printing, February 1945, pages 434-436, 440-442; published by Linde Air Products Co., New York.

70 "Welding Research Committee of The Engineering Foundation," vol. 4, No. 2, February 1940, pages 52-s to 55-s (particularly pages 52-s and 55-s).